

## UNITED STATES PATENT OFFICE

2,164,495

## OIL, GREASE, AND HYDROCARBON RESISTANT MATERIAL

Kenneth R. Brown, Tamaqua, Pa., assignor to  
Atlas Powder Company, Wilmington, Del., a  
corporation of Delaware

No Drawing. Application December 19, 1936,  
Serial No. 116,825

## 1 Claim. (Cl. 91—68)

This invention relates to oil, grease and hydrocarbon resistant material, particularly to oil, grease and hydrocarbon resistant fibrous materials, and more particularly to fibrous materials 5 carrying as a coating a flexible film, which is impervious to oils, greases and hydrocarbons, such as gasoline and the like.

The use of disposable non-refillable containers 10 for lubricating oils and particularly motor oils has become quite common in recent years. The majority of such containers are made of tinned sheet metal, but these containers are relatively expensive, difficult to seal because of the tendency of the oil to creep on the metal surface and difficult to dispose of conveniently. Moreover, when 15 such containers are emptied, a considerable portion of the oil remains within them due to its high attraction for the metal surface, entailing waste.

It has recently been proposed to use fibrous 20 containers such as containers made from paper, pulp, or the like, in place of the metal containers heretofore used. Such containers are relatively inexpensive being made from cheap materials, such as pressed waste newspaper pulp, and are 25 easily disposed of after use. Such containers are, of course, normally highly pervious to hydrocarbons, such as motor oil, and therefore, to be usable, must be provided with a flexible, inexpensive lining which is permanently impervious 30 to oil. Certain coating compositions have been proposed for use in this connection, but so far as known, none of them is entirely successful.

The principal object of this invention is the 35 production of an interiorly coated fibrous container which is highly suitable for merchandising of oils, greases and hydrocarbons.

Another object of this invention is to make an 40 oil, grease and hydrocarbon resistant material with inexpensive fibrous materials as the base, and to provide therefor an inexpensive oil, grease and hydrocarbon impervious flexible lining.

Another object of this invention is to accomplish 45 the foregoing objects by a simple and economical process.

Other objects will be apparent to those skilled 50 in the art as the description of this invention proceeds.

In the practice of the invention, there is first provided a fibrous material, such as fiber board,

cardboard, paperboard, cloth, or pressed paper pulp, and the like. Thus, if it is desired to make a container from pressed paper pulp, beaten paper pulp is pressed into the shape of the finished container by spinning or blowing into molds of desired shape. Such molds may be formed from wire screen or other foraminous or porous material, as is well understood in the art of fabricating paper pulp. A suitable container may be made from preformed cardboard or paperboard 10 if desired. Thus, sheet paper, cardboard, paperboard, pulpboard, cloth, asbestos board, asbestos paper, or the like, may be subjected to the treatment below described and supplied to the trade for use wherever oil, grease and hydrocarbon 15 resistant fibrous material is desired, or for the subsequent fabrication of containers therefrom by the usual methods known in the paper manufacture art, such as folding, cutting, and adhering with an oil, grease and hydrocarbon resistant adhesive which has an adhesive attraction for the 20 treated surfaces of the product. Within the purview of the invention, there may be used the untreated, uncoated materials above enumerated or such materials which have been treated or coated 25 with other substances than those shown below, as, for instance, rubber-impregnated or rubber-coated paper or cloth, which, of course, is subject to extremely high deterioration when left in contact with oils, greases and hydrocarbons. 30

By the term "hydrocarbon" as used in this specification and claim, it is intended to include all organic compounds containing as elements only carbon and hydrogen, including all saturated aliphatic hydrocarbons, such as gasoline, petroleum 35 naphtha, benzene, ligroin, kerosene, spindle oil, petroleum oil, such as lubricating and motor oil, mineral oil such as "Nujol", petrolatum and medicinal salves made with petrolatum as their base, lubricants containing any of the petroleum oils 40 such as soap-thickened mineral oil grease, more commonly known as "cup" grease, paraffin wax, etc., the aromatic hydrocarbons such as benzene, toluene, xylene, naphthalene, anthracene, etc., the unsaturated aliphatic hydrocarbons, such as 45 ethylene and its homologues, such as amylene, alicyclic hydrocarbons such as cyclohexane, terpene hydrocarbons such as turpentine, etc. While the invention relates primarily to liquid and semi-solid hydrocarbons, yet it is applicable 50

to solid and even gaseous hydrocarbons. Thus, material treated by the process herein disclosed might be used for the retention of gaseous hydrocarbons such as in gas-holders, gas tanks, etc.

5 By the term "oil and grease-resistant" as used in this specification and claim, there is contemplated resistance to oily and greasy hydrocarbons included in the above enumeration, as well as resistance to vegetable and animal oils 10 such as peanut butter, mayonnaise, linseed oil, hydrogenated cottonseed oil and to the higher fatty acids such as stearic acid, oleic acid, etc. In general, by the term "oil, grease and hydrocarbon-resistant" there is contemplated resistance 15 to any oily or greasy or hydrocarbon material.

It has been discovered that by the application of a plurality of coatings to the fibrous base material to be rendered oil, grease and hydrocarbon-resistant, at least one of which coatings is a cellulose derivative and at least one of which is a water-miscible organic binder such as glue or water-soluble gums flexibilized with certain sugars either alone or in combination with polyhydric alcohols, that the resulting material is highly 20 impervious to hydrocarbons, oils and greases and retains the imperviousness indefinitely. There may be used only the two coatings referred to, or other coatings in addition.

To form the cellulose derivative coating, there 30 is employed as coating material the usual lacquer made up of the cellulose derivative, suitable solvents therefor, and suitable plasticizers and softeners, but it is preferred to use an aqueous emulsion of a cellulose derivative or of 35 a cellulose derivative lacquer. As cellulose derivative, cellulose nitrate, cellulose acetate, ethyl cellulose, etc., may be used, but cellulose nitrate is preferred. A suitable formula for the emulsion which is preferred is given in the examples 40 below, but it is to be understood that other formulae and proportions may be used and that any coating of a cellulose derivative is deemed to fall within the spirit of this invention. The coating is produced by any appropriate coating 45 process. Thus, in the case of a pressed pulp container, cellulose derivative solution or emulsion may be poured into the interior and the container rotated while emptying it, allowing it to drain drip-free and drying thoroughly, preferably under forced draft conditions, and at elevated 50 temperature.

As the water-miscible organic binder there may be used any of the protein glues, such as albumin, casein, soya bean casein, zein, gelatin, 55 animal glue, hide glue or bone glue, although animal, hide or bone glue are preferred, or there may be used any of the water-soluble gums such as gum karaya, gum tragacanth, gum arabic (gum acacia), dextrine (British gum), etc. To render this film flexible there is incorporated in the initial coating composition a water-soluble sugar or a sugar syrup, such as the trisaccharides, such as raffinose, the disaccharides, such as sucrose (cane sugar), lactose, maltose, the monosaccharides, such as mannose, glucose, invert sugar (dextrose and levulose), fructose, galactose, arabinose, xylose, rhamnose, etc., or syrups of any of these sugars. For cheapness it is preferred to use the cheaper, more available sugars such as cane sugar, glucose or invert sugar. Mixtures 70 of any two or more of the enumerated sugars may be used if desired. Sugar syrups of lower purity, such as black strap molasses or "hydrol" which is an impure glucose syrup, may be used. 75 Films made from the water-miscible binder above

described flexibilized with these sugars are exceedingly impervious to hydrocarbons.

The sugars are less effective flexibilizing agents than the polyhydric alcohols, although they impart sufficient flexibility for many purposes. If desired, however, greater flexibility may be secured by using suitable proportions of the polyhydric alcohols with the sugars in compounding the water-miscible organic binder coating. Such polyhydric alcohols as ethylene glycol, diethylene 10 glycol, glycerol, xylitol, iditol, sorbitol, or technical sorbitol syrup, may be used for this purpose, preference being given to the trihydric and higher polyhydric alcohols, such as glycerol or sorbitol.

The proportions of flexibilizer and water-miscible organic binder in the coating composition are variable over a wide range. However, it is preferred to use a ratio of one to two parts of flexibilizer to one part of the binder.

The flexibilized coating may be applied by any 20 known coating process. Thus, it may be applied to preformed containers in the same manner as above described for the cellulose derivative coating, but it is preferable to heat it before coating with it.

Oil, grease and hydrocarbon resistance is obtained in the product whether there is first applied the cellulose derivative coating, followed by the flexibilized water-miscible organic coating, or whether the coatings are applied in the 20 reverse order with the flexibilized water-miscible organic coating next to the base material and superimposed thereupon the cellulose derivative coating. However, the first mentioned order is preferred, especially when using an aqueous cellulose derivative lacquer emulsion on a fibrous base since the water of the emulsion is taken up by the porous base material very rapidly, resulting in a high adherence of the lacquer, and a very much shortened drying time is necessary 40 before the flexibilized coating is applied. Moreover, containers so prepared in which the oil-repellant coat is in direct contact with the hydrocarbon oil drain more completely on emptying. The flexibilized water-miscible organic binder 45 coat shows such a high adherence to the cellulose derivative undercoat that the two coats cannot be separated. The cellulose derivative undercoat protects the water-miscible organic film from atmospheric moisture or dryness which 50 might penetrate through the fiber base, while the water-miscible organic coating protects the cellulose derivative undercoat from contact with the oil, grease or hydrocarbon material which 55 might tend to dissolve the plasticizer therefrom, resulting in leakage. Thus, it is seen that the dissimilar coats described cooperate in a new and novel manner and produce results which 60 would not be obtainable with two cellulose derivative coats or two water-miscible organic coats. Moreover, a more economical coating is obtained using the coatings described. However, with water-miscible organic binder as the first coat, and cellulose derivative as the second coat, many of the advantages of the invention 65 are attained and the container will not fail altogether in humid climates.

When reference is made to sorbitol, there is also contemplated a technical grade of sorbitol syrup prepared by the catalytic hydrogenation 70 or electrolytic reduction of glucose and which may contain as impurities some unreduced glucose, ash and salts of organic acids.

In the following examples there are set forth several preferred embodiments of the invention. 75

It is to be understood, however, that the invention is not limited thereto.

## EXAMPLE 1

|                                   |                                  |                                      |
|-----------------------------------|----------------------------------|--------------------------------------|
| 5                                 | Coating A (cellulose derivative) | 5                                    |
| Water phase, 28½% by weight       | Per cent by weight               | Per cent by weight                   |
| 10 Water                          | 99                               | (dry basis)                          |
| Sulfonated castor oil (75% grade) | 1                                | Invert sugar syrup (50% inverted) 15 |

100 Grams per gallon

|                                                                                        |      |                                         |
|----------------------------------------------------------------------------------------|------|-----------------------------------------|
| 15 Sodium salt of sulfonated lauryl alcohol extracted with methyl alcohol (Duponol Me) | 19   | Hide glue (gel. strength 400-415 g.) 15 |
| Methyl cellulose (Tylose S-25)                                                         | 11.4 | Water 10                                |

20 Lacquer phase, 71½% by weight

|                    |                    |                                         |
|--------------------|--------------------|-----------------------------------------|
| Liquids, 1 gallon. | Per cent by volume | Per cent by weight                      |
| Octyl acetate      | 5                  | Cane sugar 7.5                          |
| Butyl acetate      | 30                 | Glycerine 7.5                           |
| 25 Butyl alcohol   | 10                 | Hide glue (gel. strength 400-415 g.) 25 |
| Toluol             | 21                 | Water 15.0                              |
| Blown castor oil   | 34                 | 70.0                                    |

30 Solids.

Nitrocellulose (7 sec.) oz. 25

The water phase is prepared by dissolving the sulfonated castor oil in the distilled water, then adding to one gallon of the resulting solution the sodium salt of sulfonated lauryl alcohol and the methyl cellulose in the proportion stated. The lacquer phase is made by dissolving the nitrocellulose in the previously prepared mixture of solvents and plasticizer. The given proportion of lacquer phase is then emulsified in the water phase by passing the mixture through a colloid mill or homogenizer.

## 45 Coating B (glue)

|                      |                    |                                      |
|----------------------|--------------------|--------------------------------------|
| 45                   | Coating B (glue)   | 45                                   |
| Per cent by weight   | Per cent by weight | Per cent by weight                   |
| Crystallized glucose | 15                 | Invert sugar syrup (50% inverted) 13 |

Hide glue (gel. strength 400-415 g.) 15

Water 70

50 The crystallized glucose and water are heated in a jacketed kettle with agitation to 170° F. The glue is added and heating is continued between 170° and 180° F. until the mixture is uniform and grain-free. The water removed by evaporation is replaced. Preferably 1% of beta naphthol on the weight of the glue or similar anti-mold compound is added.

55 A container of pressed paper pulp sized throughout during manufacture with 10% of paraffin wax is first coated with Coating A by filling the container with the lacquer emulsion and immediately pouring it out with a rotary motion. The excess is allowed to drain drip free and the container is then dried for 15 minutes at 150-160° F. or for 2 hours at 120-130° F. in a drying chamber equipped with a fan for circulating the air. The container is then removed and coated with Coating B which is applied at a temperature of 160-180° F., the manner of application being otherwise identical with that of Coating A. The container is then dried for 16 hours at room temperature and then dried 2 hours at 150-160° F. in the same type of drying chamber as described above.

## EXAMPLE 2

## Coating A

The same as in Example 1.

## Coating B (glue)

|                                      |                  |                                         |
|--------------------------------------|------------------|-----------------------------------------|
| 5                                    | Coating B (glue) | 5                                       |
| Per cent by weight                   | (dry basis)      | Per cent by weight                      |
| Invert sugar syrup (50% inverted)    | 15               | Invert sugar syrup (50% inverted) 15    |
| Hide glue (gel. strength 400-415 g.) | 15               | Hide glue (gel. strength 400-415 g.) 15 |

The coatings are prepared and applied to the paper pulp container in exactly the same manner as that described in Example 1.

15

## EXAMPLE 3

## Coating A

The same as in Example 1.

## Coating B

|                                      |                    |                                           |
|--------------------------------------|--------------------|-------------------------------------------|
| 20                                   | Coating B          | 20                                        |
| Per cent by weight                   | Per cent by weight | Per cent by weight                        |
| Cane sugar                           | 7.5                | Cane sugar 7.5                            |
| Glycerine                            | 7.5                | Glycerine 25                              |
| Hide glue (gel. strength 400-415 g.) | 15.0               | Hide glue (gel. strength 400-415 g.) 15.0 |

The coatings are prepared and applied to the paper pulp container in exactly the same manner as that described in Example 1. In making up Coating B the glycerine, cane sugar and water are first heated, the glue being added later.

## EXAMPLE 4

## Coating A

The same as in Example 1.

## Coating B

|                                   |                    |                                      |
|-----------------------------------|--------------------|--------------------------------------|
| 40                                | Coating B          | 40                                   |
| Per cent by weight                | Per cent by weight | Per cent by weight                   |
| (dry basis)                       | (dry basis)        | (dry basis)                          |
| Invert sugar syrup (50% inverted) | 13                 | Invert sugar syrup (50% inverted) 13 |
| Casein                            | 12                 | Casein 12                            |
| Ammonia, 26°                      | 1                  | Ammonia, 26° 1                       |
| Water                             | 45                 | Water 45                             |

Weigh the water (less the water in the sugar syrup) into an agitated, jacketed kettle and add the casein, stirring until all lumps are dispersed. Add the ammonia and heat slowly (in the course of 40 minutes) with stirring to 160° F. Add the invert sugar syrup and stir at 150-160° F. until homogeneous. Replace evaporated water.

The coatings are applied in exactly the same manner as in Example 1, except that Coating B should be applied at a temperature not exceeding 160° F.

The fibrous containers produced as in Examples 1 to 4 are extremely impervious to hydrocarbons and are especially adapted for use as non-refillable containers for dispensing motor and lubricating oils. The use of pressed paper pulp for such containers is extremely advantageous since it is cheap and seamless. While reference has been made to containers made from such pulp sized with wax, it will be obvious that containers made from unsized pulp or from pulp sized with other agents, such as 5% of rosin size, may be used.

70

## EXAMPLE 5

## Coating A

The same as in Example 1.

75

## Coating B

|                                        | Per cent by weight |
|----------------------------------------|--------------------|
| Glucose                                | 7.5                |
| Glycerol                               | 7.5                |
| 5 Hide glue (gel. strength 400-415 g.) | 15.0               |
| Water                                  | 70.0               |

This coating is made up as in Example 3, the glycerol, glucose and water being first heated to 10 170° and the glue being then added.

10 Coating A is first uniformly applied by spraying on 16 oz. cotton duck. The coated fabric is dried at 150-160° F. for thirty minutes. Then Coating B at a temperature of 150-160° F., is sprayed uniformly as a second coat and dried at 15 150-160° F. for two hours. The fabric thus prepared is extremely resistant to penetration by hydrocarbons, and, for example, may be used in the fabrication of hose or tubing through which 20 gasoline or other hydrocarbons are to be passed.

## EXAMPLE 6

## Coating A

26 The same as in Example 1.

## Coating B

The same as in Example 1. Asbestos paper is sprayed with coatings A and B exactly as in Example 5. The product is extremely oil-resistant, 30 and may be used as gasket material where oil resistance is a prime requisite, provided the temperature to which it is subjected does not exceed 150° F.

## EXAMPLE 7 (DEXTRINE FLEXIBILIZED WITH 35 DEXTROSE)

## Coating A

40 The same as in Example 1.

## Coating B

|                    | Per cent by weight |
|--------------------|--------------------|
| Dextrose           | 25                 |
| White corn dextrin | 25                 |
| Water              | 50                 |

45 This coating was made up by commingling the specified materials and subjecting them to slight heating while agitating in order to obtain a homogeneous mixture.

50 Coating A was applied to a paper pulp cone exactly as in Example 1. Coating B was then applied over Coating A by a dipping operation, followed by draining drip-free, whereupon the container was dried for 2 hours at 140-150° F.

## EXAMPLE 8 (DEXTRINE FLEXIBILIZED WITH GLUCOSE)

55 This example is exactly like Example 7 except that 25% of hydrol on the dry basis was substituted for the dextrose in that example. Hydrol is an impure glucose syrup.

## EXAMPLE 9 (DEXTRINE FLEXIBILIZED WITH INVERT SUGAR)

60 This example is exactly like Example 7 except that 25% of Nulomoline (dry basis) was substituted for the dextrose in that example. Nulomoline is an impure invert sugar syrup comprising dextrose and levulose.

65 As will be apparent to those skilled in the art, if oil, grease or hydrocarbon resistance is desired in a portion only of a container or surface, only that portion is treated by the process herein disclosed.

70 It is also to be understood that it is not desired to be limited to the above description and specific 75 examples. Thus, any lacquer or lacquer emulsion

comprising a cellulose derivative may be used. Any cellulose ester or ether may be used. Other plasticizers and solvents than those shown may be used. Compatible resins, either natural or synthetic, may be added to the cellulose derivative coating composition. The coats may be applied in any suitable manner. The proportion of ingredients, order of mixing and temperatures of application, may all be varied considerably without departing from the spirit of the invention. Thus, 10 if desired, instead of the drying procedure described for Coating B in the examples, the coating of the superimposed glue may be dried at atmospheric temperature for a period of from 15 minutes to twenty-four hours, preferably for 16 hours, 15 before being placed in the oven, in order to allow the melting point of the glue mixture to rise above that of the drying oven by evaporation of water, or formaldehyde or paraformaldehyde may be added in the glue mix so as to set the glue coating 20 before drying, or the glue-coating may be sprayed with aqueous formaldehyde after its application and prior to drying. When formaldehyde is used in glue coat, it is highly preferred to use 14-16% of 100% formaldehyde (CH<sub>2</sub>O) calculated on the 25 weight of the glue. If desired, drying of the glue coat at elevated temperatures may be altogether eliminated by the use of the specified proportion of formaldehyde and by the expedient of drying at room temperature for 16 hours. Other drying 30 temperatures than those specified in the examples may be used if desired. The coatings described in the examples may be used interchangeably. Thus, pressed paper pulp might be used as the base in Example 5, or fabric as the base in Examples 1 to 4.

35 By "oil, grease and hydrocarbon-resistant" as used in the claim is meant impermeable to and not decomposed by or chemically affected by oils, 40 greases and hydrocarbons generally, including those herein enumerated. It is not intended to be limited to such hydrocarbons as gasoline and motor oil to which the invention is particularly applicable. By "water-miscible organic binder" as used in the claim, there is meant water-miscible organic binders of the type herein disclosed and similar materials, namely, protein glues such as hide or bone glue or casein, or the water-soluble gums such as gum arabic, dextrine, etc. These binders are of the type that form solutions or colloidal suspensions upon admixture with water. By "glue" there is meant protein glues such as hide and bone glue, gelatine, casein, albumin, etc. By "water-soluble gum" is meant such natural gums as are herein disclosed, dextrine and similar gums which are termed "water-soluble" by those skilled in the arts. The terms "a cellulose derivative", "a water-miscible organic binder", and "a water-soluble gum" are intended to cover single or mixed ingredients falling within 45 these expressions.

In co-pending application, Serial Number 112,014 filed November 21, 1936, there is disclosed the use of a water-miscible organic binder coating flexibilized with polyhydric alcohols in conjunction with a cellulose derivative coating for rendering materials oil, grease and hydrocarbon-resistant. In co-pending application, Serial Number 111,599, filed Nov. 19, 1936, there is disclosed a coating composition comprising a water-miscible 50 organic binder flexibilized with sorbitol or mixtures of sorbitol and lower polyhydric alcohols.

55 Having described my invention, what I claim is:

An oil, grease and hydrocarbon-resistant fibrous material comprising a fibrous base provided with 75

two superimposed flexible coatings, the first coating which is in contact with the fibrous base being highly resistant to moisture and consisting essentially of a plasticized cellulose derivative, and the second coating which is superimposed over said first coating and which is to be exposed to oil, grease or hydrocarbon being highly resistant to oils, greases and hydrocarbons and consisting

essentially of a water-miscible organic binder selected from the group consisting of protein glues and water-soluble gums flexibilized with substantially an equal amount of a flexibilizer containing at least 50% of water-soluble sugar, said flexibilizer being selected from the group consisting of water-soluble sugars and polyhydric alcohols.

KENNETH R. BROWN.